

## UNITED STATES PATENT OFFICE

2,066,582

ULTRAVIOLET PRINTING-OUT  
COMPOUNDS

Samuel E. Sheppard and Waldemar Vanselow,  
Rochester, N. Y., assignors, by mesne assignments,  
to Eastman Kodak Company, Jersey  
City, N. J., a corporation of New Jersey

No Drawing. Application September 7, 1935,  
Serial No. 39,626

4 Claims. (Cl. 95—7)

This invention relates to photographically sensitive materials and more particularly to such materials containing the silver salts of certain pyrazolone compounds and useful for printing out purposes when exposed to ultra-violet light.

Light-sensitive papers of the type which exhibit a visible image directly on exposure to light, without subsequent development, are known as "printing-out" papers. Such papers are useful 10 in recording the intensity of light or the duration of exposure, as in actinometers, exposure meters, automatic recording machines, etc. These papers are usually sensitive mainly to visible light, and continue to change color on long 15 exposure to ordinary illumination. When the intensity of light of shorter wave is to be measured, or when the exposed material is to be subjected to conditions of slight illumination, it is desirable to have a material which is relatively insensitive 20 to visible light, and sensitive mainly to the rays to be measured.

It is accordingly the principal object of the present invention to provide a light-sensitive material which is sensitive to ultra-violet light, and 25 relatively insensitive to visible light.

This object is accomplished by the present invention by sensitizing a colloidal material with a silver salt of certain pyrazolone compounds.

The methods by which these materials are 30 made and their properties will now be described.

*I.—Silver salt of 1-p-sulfo-phenyl-3-methyl-5-pyrazolone*

A water solution of 1.7 grams of silver nitrate 35 in 20 c. c. of 5% gelatin was added slowly but with vigorous stirring to a gelatin solution of 2.5 grams of 1-p-sulfo-phenyl-3-methyl-5-pyrazolone. The pyrazolone was dissolved in 200 c. c. of water and then to this water solution were 40 added 200 c. c. of a 10% gelatin sol. In the course of several minutes the emulsion assumed a tan color which would turn black if exposed to dull daylight. The emulsion was prepared in the light of a safelight transmitting orange and red 45 light. Gelatin coated paper was coated with the emulsion of the silver pyrazolone and allowed to dry. The paper is sensitive to ultra-violet light, giving a purple print-out on a pale tan ground. Heating to 80° C. has no effect on the unfixed 50 print.

*II.—Silver salt of 4-sulfo-phenyl-3-carboxylic acid-5-pyrazolone*

50 c. c. of a 1% gelatin solution containing 1.7 55 grams of silver nitrate was added to 200 c. c. of

a 5% gelatin solution containing 2.8 grams of 4-sulfo-phenyl-3-carboxylic acid-5-pyrazolone. A cream colored emulsion which was very viscous was obtained. Paper was coated by spreading the emulsion by force. Even if the gelatin 5 is entirely omitted, a syrupy sol. of the silver pyrazolone is obtained. The paper is sensitive to daylight but more so to ultra-violet light wherein it turns dark red brown in color. Heating to 80° C. has no effect on the unfixed print. 10

*III.—Silver salt of 1-phenyl-3-carboxylic acid-5-pyrazolone*

50 c. c. of a 5% gelatin solution containing 1.7 grams of silver nitrate was added to 200 c. c. of 15 a 5% gelatin solution which was saturated with 1-phenyl-3-carboxylic acid-5-pyrazolone (which contained less than 3 grams of the pyrazolone). A cream colored emulsion was obtained after allowing it to stand for several minutes. Paper 20 was coated as before. Exposure to ultra-violet light produces a purple image on a pale brown ground.

The image of the unfixed print can be intensified by heating it to 80° C. However, the ground 25 also becomes somewhat darker upon heating.

*IV.—Silver salt of meta-nitrophenyl pyrazolone carboxylic acid*

The procedure as described for the preparation 30 of the silver salt of 1-phenyl-3-carboxylic acid-5-pyrazolone was followed. Upon exposure to the ultra-violet light a pale purple image on a pale yellow ground is obtained. Heating has no intensifying action on the image but does cause 35 the entire gelatin layer to rise (become thicker).

In every case the unaffected salt can be removed in sodium thiosulfate thus offering a means of fixation of the print. The layer is relatively 40 insensitive to visible light so that fixing is not necessary when the prints are kept in conditions of ordinary indoor illumination.

What we claim is:

1. A photographic material sensitive to ultra-violet light and comprising a colloid carrier and 45 a photo-sensitive material, the sensitive material being a silver salt of one of the following pyrazolone compounds: 1-p-sulfo-phenyl-3-methyl-5-pyrazolone, 4-sulfo-phenyl-3-carboxylic acid-5-pyrazolone, 1-phenyl-3-carboxylic acid-5-pyrazolone, and meta-nitrophenyl pyrazolone carboxylic acid. 50

2. A photographic material sensitive to ultra-violet light and comprising a colloid carrier and 55 a photosensitive material, the sensitive material

being a silver salt of 1-p-sulfo-phenyl-3-methyl-5-pyrazolone.

3. A photographic material sensitive to ultra-violet light and comprising a colloid carrier and 5 a photosensitive material, the sensitive material being a silver salt of 4-sulfo-phenyl-3-carboxylic acid-5-pyrazolone.

4. A photographic material sensitive to ultra-violet light and comprising a colloid carrier and a photosensitive material, the sensitive material being a silver salt of 1-phenyl-3-carboxylic acid-5-pyrazolone.

5

SAMUEL E. SHEPPARD.  
WALDEMAR VANSELOW.